# EUROPEAN PATENT SPECIFICATION

(11) **EP 3 168 319 B1**
(45) Date of publication and mention of the grant of the patent: **16.12.2020**
(21) Application number: 14897352.2
(22) Date of filing: 08.07.2014
(51) Int. Cl.: C22C 38/02, C22C 38/04, C21C 7/064, C21C 7/10, C22C 38/00, C22C 38/06, C22C 38/42, C22C 38/44, C22C 38/46, C22C 38/48, C22C 38/50

(54) **MICROALLOYED STEEL FOR HEAT-FORMING HIGH-RESISTANCE AND HIGH-YIELD-STRENGTH PARTS**
MIKROLEGIERTER STAHL ZUM WARMFORMEN VON HOCHBESTÄNDIGEN TEILEN MIT HOHER STRECKGRENZE
ACIER HAUTE RÉSISTANCE FAIBLEMENT ALLIÉ POUR FORMAGE À CHAUD DE PIÈCES DE HAUTE RÉSISTANCE ET DE LIMITE ÉLASTIQUE ÉLEVÉE

(43) Date of publication of application: 17.05.2017
(73) Proprietor: Sidenor Investigación y Desarrollo, S.A., 48970 Elexalde-Basauri (Bizkaia) (ES)
(72) Inventor: IDOYAGA OLANO, Zuriñe, E-48970 Elexalde-Basauri (Vizcaya) (ES); ALBARRÁN SANZ, Jacinto José, E-48970 Elexalde-Basauri (Vizcaya) (ES); CANTERO VIQUIERA, Oihane, E-48970 Elexalde-Basauri (Vizcaya) (ES); LARAUDOGOITIA ELORTEGUI, Juan José, E-48970 Elexalde-Basauri (Vizcaya) (ES)
(74) Representative: Herrero & Asociados, S.L.
(86) International application number: PCT/ES2014/070558
(87) International publication number: WO 2016/005615

(56) References cited:
- EP-A1- 1 568 792
- EP-A1- 2 057 298
- EP-A1- 2 159 296
- EP-A1- 2 524 970
- WO-A1-2013/121930
- ES-T3- 2 302 935
- FR-A1- 2 833 617
- JP-A- H06 287 677
- JP-A- H10 121 200
- SEROSH ENGINEER ET AL: "A review of the development and application of microalloyed medium car- bon steels", STEEL RESEARCH INTERNATIONAL, vol. 58, no. 8, 2 August 1987 (1987-08-02) , pages 369-376, XP055600442,

## Description

### Object of the Invention

The present invention relates to a high-strength and high-yield strength microalloyed steel.

The invention allows producing a microalloyed steel with high mechanical strength and high yield strength, in addition to responding well to machining operations, based on a given chemical composition, a specific metallurgical process and subsequent controlled cooling.

### Background of the Invention

Microalloyed steel is basically classic building steel to which small amounts of alloy elements, such as V, Al, Ti, Nb, Zr, B, etc., capable of forming microprecipitates are added.

The main characteristic of microalloyed steels is based on the occurrence of microprecipitates produced during both the rolling process and the forging process. It is therefore necessary to know the formation and evolution of microprecipitates as a function of thermal cycles, hot deformations and cooling rates in order to dominate the process and produce steel with the desired mechanical properties.

One of the main applications of microalloyed steels are certain automotive engine components, such as the crankshaft, connecting rods, the rail of common-rail, etc. All these elements are components subjected to high working pressures and stresses, so it is fundamental for them to have very high tensile strength and yield strength values.

The advantage with respect to quenched and tempered steels they are replacing is based on the fact that these microalloyed steels acquire characteristics directly by means of thermomechanical treatment and subsequent controlled cooling.

The microalloyed steels of the present patent have a ferrite-perlite structure, and their final application is in heat-forming.

On the other hand, the machinability of microalloyed steel after a heat-forming process is comparable to that of quenched and tempered steel, provided that they both have similar hardness and sulfur content levels.

The main advantage derived from the use of microalloyed steels is the direct reduction of the cost of the formed components up to 10-20%, primarily due to the simplification of the manufacturing process by eliminating thermal treatment from quenching and tempering, as well as subsequent straightening operations, stress relief operations, as well as hardening cracks and controls for detecting them.

Different microalloyed steel grades are used today according to the strength to be attained in components for which they are going to be used. The characteristics are largely determined by the carbon content of the steel, which can range between 0.15% and 0.50% by weight, as well as the content of other alloying elements, such as Mn and Si, for example, which help with solid solution hardening of ferrite and other microalloying elements such as Ti, V and, in some cases, Nb as well, which form carbide and nitride microprecipitates, functioning as controllers of grain size and precipitation hardening.

The different microalloyed steel grades manufactured today range from 550 MPa to 1000 MPa in terms of strength. These values considerably depend on the thickness of the part and on the forming process and subsequent cooling to which the part is subjected.

There are different patents today related to microalloyed steels. Several examples are mentioned below.

Patent application no. CN102776439(A)2012 "Niobium microalloying Si-Mn-B series hot forming steel plate and rolling technology" describes a microalloyed steel with Nb but for a flat product with a mechanical strength between 700-900 MPa and a yield strength of 500-600 MPa.

Patent application no. CN101629268(A)2010 "Microalloying high-strength and anti-crack flat steel for automobile girder and production process thereof" describes a microalloyed steel in V producing an as-rolled product between 750-850 MPa and a yield strength between 640-700 MPa.

Patent application no. CN101307413(A)2008 "Microalloying steel for ultrahigh-strength sucker rod" describes a microalloyed steel with Nb, Ti and V for rods, with a tensile strength greater than 965 MPa.

Patent application n° EP2816131 relates to a rolled steel bar for hot forging suitable as a starting material for a common rail used for a diesel engine fuel injection system, a hot forged section material produced by forming the rolled steel bar, the common rail and the method for producing the common rail. The Nb is not present in the rolled steel bar described.

Patent application n° EP2159296 refers to a quench hardened and tempered steel and to a method for obtaining parts of said steel. The Nb is not present in the composition of the steel. JPH10121200 discloses a high strength steel material for shear reinforcing bar, excellent in bendability and weldability having a specific composition containing specific amounts of Nb and V and also having a structure composed of ferrite and pearlite.

Therefore, there is no microalloyed steel in the state of the art with a tensile strength exceeding 1000 MPa.

### Description of the Invention

The present invention relates to microalloyed steel for forming high-strength and high-yield strength parts as defined in Claim 1. The steel of the invention consists of a ferrite-perlite structure with mechanical characteristics in which the tensile strength is 1050-1200 MPa, depending on the diameter of the bar and the yield strength is greater than 750 MPa.

The invention allows producing a microalloyed steel from a novel chemical composition and a given metallurgical process, having high mechanical strength while at the same time high yield strength, which is fundamental for all automotive components.

The thermomechanical treatment to which the component formed with the steel in question is subjected has a very important influence on the microstructure, and therefore on the mechanical characteristics of the end component, i.e., the steel with the initial chemical composition must be formed under given conditions and be subjected to controlled cooling under certain conditions in order to achieve the optimized mechanical characteristics of the end component.

In order to assure good mechanical characteristics which in turn entail a long fatigue life, a specific deoxidation and inclusions separation method in given special conditions must be applied during the manufacturing process for producing this steel.

A synergistic effect has been found between a novel combination of chemical elements and a method of controlled cooling to obtain the characteristics required for said steel.

In turn, since most of the automotive components for which this steel has been designed require significant machining operations after the forging process, the chemical composition of this steel is designed so that its post-forming process machinability is comparable to or even better than that of classic quenched and tempered steel when they both have similar hardness and sulfur content levels.

The research that was conducted resulted in a new SiMnV alloyed steel grade, with the composition disclosed in claim 1.

These alloy elements are used in microalloyed steels to improve the tensile strength and other characteristics that allow the use thereof in the discussed applications.

Each of the alloy elements, in the proportions indicated above, has an influence on given parameters and properties of the steel that is finally produced.

Carbon is an essential element for obtaining high strength and hardness, as well as a long fatigue life. In the microalloyed steels, carbon tends to form carbides, hardening and providing strength to said steels.

In addition to being a strong deoxidizer, silicon provides solid solution hardening as it dissolves into the ferrite matrix.

Manganese prevents the detrimental effect of sulfur, combining with it to form MnS and thereby improving machinability. On the other hand, like silicon, manganese dissolves in the ferrite crystalline network, replacing the iron atoms and causing solid solution hardening.

Vanadium is a microalloying element that contributes to refining the grain size and when it combines with carbon, it forms vanadium carbides, which bring about intense precipitation hardening. Vanadium precipitates are hydrogen nucleators, such that in corrosive environments they fix it and improve hydrogen-induced delayed fracture resistance. However, with very high vanadium contents the precipitates coalesce and their effect can become detrimental. Therefore, the optimal vanadium content is between 0.05% and 0.50%.

Niobium is a microalloying element having effects similar to those of vanadium on grain size control and on precipitation hardening of the steel, such that it contributes to increasing the mechanical strength and to improving toughness. Furthermore, niobium precipitates fix the hydrogen attacking the steel in corrosive environments, improving the delayed fracture resistance. At more than 0.050%, nevertheless, the precipitates swell, which is detrimental for the mechanical properties, in addition to increasing the risk of the occurrence of bainites. The optimal niobium content is set between 0.001% and 0.050%.

Furthermore, it is contemplated that the steel proposed by the invention may additionally comprise at least one of the following elements, or a combination thereof, in percentage by weight:
P ≤ 0.015%
S ≤ 0.10%
Cr ≤ 0.50%
Ni ≤ 0.50%
Mo ≤ 0.10%
Cu ≤ 0.25%
0.001% ≤ Al ≤ 0.050%
0.004% ≤ N ≤ 0.020%

Phosphorus hardens the steel and segregates at the austenite grain boundaries, drastically reducing the toughness of the steel. Furthermore, it favors hydrogen embrittlement and delayed fracture. In order to limit its adverse effect, the phosphorus content is limited to less than 0.015%.

Sulfur embrittles steel similarly to phosphorus. Despite the fact that this effect is counteracted by combining with manganese, manganese sulfides form inclusions which deform longitudinally in the forging or rolling direction and considerably deteriorate transverse mechanical properties and fatigue behavior. However, sulfur must be added in small amounts because it brings about microalloyed steel machinability improvements, hence the content thereof being limited to 0.10%.

Chromium is an essential element for assuring steel quenchability; however, since a ferrite-perlite structure is desired for the microalloyed steel of the invention, chromium is an element that must be controlled, hence it is limited to a maximum of 0.50%.

Nickel is an element which, at high concentrations, inhibits ferrite formation and furthermore favors quenchability; hence, like chromium, nickel is an element that must be controlled in microalloyed steels. For that reason, it must be limited to a maximum of 0.50%

Molybdenum has an effect which greatly favors quenchability, just like chromium and even more than nickel; hence, for a microalloyed steel with a ferrite-perlite structure it is limited to a maximum of 0.10%.

The addition of copper prevents steel decarburization and improves corrosion resistance in a manner similar to nickel, inhibiting the growth of corrosion pits. However, a high copper content impairs hot ductility of the steel such that the upper limit of copper is set at 0.25%.

Aluminum is an element that acts like a strong deoxidizer during the steel manufacturing process. Aluminum forms aluminum nitrides which contribute to controlling austenite grain size during heating prior to heat-forming processes. Nevertheless, it forms very hard oxides that are highly detrimental for fatigue life, such that the upper limit thereof is set at less than 0.050%.

Nitrogen combines with Ti, Nb, Al and V to form nitrides, the precipitation temperatures of which depend on the respective content of the different elements and on constant features. With a suitable size, those nitrides exert a pinning effect on the austenite grain by controlling its size at a high temperature and preventing coalescence and growth thereof. However, if the nitrogen or microalloying element content is very high, precipitation occurs at a high temperature and the precipitates swell, being rendered ineffective for controlling grain and detrimental for the fatigue life. As a result, the nitrogen content in the steel is limited to 0.004% to 0.020%.

Therefore, after various experiments a rigorous method for producing steel comprising the following steps has been developed:
- Rigorously controlling the raw materials from the furnace.
- Performing an oxidation period in an electric furnace, which is important for dephosphorization of the steel, prior to foamed slag.
- Once foamed slag has ended, deslagging is performed until rendering the furnace virtually slag-free, the objective being a presence of phosphorus in this step less than 0.007% by weight.
- Tipping until overturning with standard temperature and parts per million (ppm) of oxygen, making sure that slag does not go from the furnace to the ladle.
- Generating a prolonged vacuum, a vacuum below 1 mbar being considered the vacuum time.
- Ending the vacuum treatment with sufficient temperature to perform an inclusion separation process after same lasting at least fifteen minutes, without performing additions or heating of any type.
- Finally, a meticulous casting process must be followed with special protection of the liquid steel stream.
- If the solidification process is in continuous casting, the casting speed, cooling and stirring conditions will be adjusted for producing a microstructure with homogenous solidification.
- Providing a suitable design of the secondary cooling, as well as a slow tertiary cooling, in order to prevent thermomechanical stresses that may result in the occurrence of cracks.
- Reaching the straightening at a temperature above the temperatures at which hot ductility decreases for these steels.

This entire method of manufacturing the steel allows achieving the desired sulfur levels and phosphorus levels below 0.015% by weight, in addition to a low inclusion level.

The CCT (continuous cooling transformation) diagrams allow knowing the cooling rates suitable for obtaining a ferrite-perlite microstructure in the steel according to the invention.

The solidification products are later transformed in heat conditions by means of a process that consists of heating at a temperature between 900-1300°C and a series of consecutive deformations by means of hot forging or rolling until producing an intermediate product having a suitable section, shape and microstructure.

After various experimental tests, it was found that after the process of manufacturing the steel disclosed herein, with the chemical composition indicated above and adjusting the cooling rates after the forging or rolling process, a steel having a ferrite-perlite structure, with a tensile strength between 1050 and 1200 MPa, depending on the section of the bar or component, is achieved.

To produce a component made of the steel previously produced having the mentioned features, the disclosure contemplates the possibility of carrying out a method whereby said steel part can be produced. Said possibility comprises, after producing the steel, the following steps:
- manufacturing a component made of said steel,
- performing controlled cooling of the component immediately after heat-forming,
- machining the component with its final geometry.

Therefore, according to the disclosure the method for producing parts made of said steel comprises a heat-forming process, with prior heating at a temperature between 900-1300°C, which allows providing the steel with sufficient hot ductility, in order to give the part of steel a shape similar to that of the end component. After shaping, the part is subjected to controlled cooling, which will allow achieving the desired mechanical characteristics with a 100% ferrite-perlite structure.

It is subsequently contemplated that said disclosure of the method for manufacturing the microalloyed steel part comprises a machining process machining to obtain the final geometry of the component, hence in order to improve the response of the steel with respect to machinability, the steel can possibly have elements such as sulfur and other elements for improving machinability.

Therefore, it is contemplated that a disclosure of the method for producing steel parts comprises the following steps:
- Manufacturing the steel of the invention described above, in which the selected steel comprises the general composition or the preferred composition defined above.
- Process of rolling the steel in question.
- Manufacturing a part made of said steel by means of a heat-forming process.
- Controlled cooling of the part after heat-forming.
- Machining operations on the formed part.

### Description of the Drawings

To complement the description that is being made and for the purpose of helping to better understand the features of the invention according to a reference example thereof, a set of drawings is attached as an integral part of said description, in which the following is depicted with an illustrative and nonlimiting character:
Figure 1 shows a table, divided into Figures 1a and 1b, comprising photographs of the microstructures obtained after heat-forming for the same part in the samples of steels A-G defined in Table 1.
Figure 2 shows photographs of the microstructures in which details of the bainites found in castings B, C, D and E can be seen.

### Reference examples not according to the invention

By way of example, the tests conducted with samples of steels with other compositions different from the chemical composition of the steel of the invention are described below. Table 1 shows the chemical compositions in percentage by weight, the rest being iron and impurities:

**Table 1**

| | C | Mn | Si | P | S | Cr | Ni | Mo | V | Cu | Al | Ti | N* |
|---|---|---|---|---|---|---|---|---|---|---|---|---|---|
| A | 0.36 | 1.05 | 0.72 | 0.009 | 0.023 | 0.12 | 0.09 | 0.020 | 0.26 | 0.13 | 0.019 | 0.025 | 152 |
| B | 0.38 | 1.37 | 0.72 | 0.009 | 0.069 | 0.15 | 0.14 | 0.032 | 0.25 | 0.21 | 0.010 | 0.009 | 136 |
| C | 0.37 | 1.39 | 0.95 | 0.012 | 0.073 | 0.13 | 0.14 | 0.034 | 0.26 | 0.21 | 0.008 | 0.009 | 207 |
| D | 0.40 | 1.40 | 1.28 | 0.010 | 0.060 | 0.19 | 0.13 | 0.033 | 0.26 | 0.20 | 0.004 | 0.006 | 95 |
| E | 0.40 | 1.42 | 1.51 | 0.010 | 0.062 | 0.18 | 0.13 | 0.033 | 0.25 | 0.21 | 0.004 | 0.006 | 99 |
| F | 0.40 | 1.16 | 1.06 | 0.007 | 0.063 | 0.15 | 0.12 | 0.028 | 0.25 | 0.07 | 0.009 | 0.014 | 133 |
| G | 0.44 | 1.40 | 0.40 | 0.011 | 0.070 | 0.21 | 0.06 | 0.020 | 0.12 | 0.10 | 0.017 | 0.016 | 137 |
| H | 0.44 | 1.21 | 0.91 | 0.008 | 0.025 | 0.09 | 0.08 | 0.012 | 0.26 | .010 | 0.011 | 0.013 | 162 |

| | | | | | | | | | | | | | |
|---|---|---|---|---|---|---|---|---|---|---|---|---|---|
| (*) ppm | | | | | | | | | | | | | |

Table 2 shows the values of the mechanical characteristics obtained for one and the same component already formed with all the castings of Table 1.

**Table 2**

| | Yield strength (MPa) | Tensile strength (MPa) | Elongation (%) | Reduction (%) |
|---|---|---|---|---|
| A | 698 | 954 | 18 | 48 |
| B | 824 | 1102 | 13 | 25 |
| C | 779 | 1056 | 9 | 18 |
| D | 880 | 1140 | 10 | 38 |
| E | 887 | 1141 | 8 | 32 |
| F | 740 | 1016 | 18 | 40 |
| G | 648 | 956 | 21 | 41 |
| H | 804 | 1118 | 15 | 35 |

It can be seen that steels B-C-D and E have exceeded a strength of 1050 MPa and yield strength of 750 MPa; however, the microstructure of these steels after heat-forming has shown traces of bainites.

The following table shows the different percentages of phases found in the different components with the castings of Table 1.

**Table 3**

| | Ferrite (%) | Perlite (%) | Bainite (%) |
|---|---|---|---|
| A | 40 | 60 | 0 |
| B | 10 | 65 | 25 |
| C | 15 | 75 | 10 |
| D | 20 | 75 | 5 |
| E | 15 | 80 | 5 |
| F | 40 | 60 | 0 |
| G | 35 | 65 | 0 |
| H | 35 | 65 | 0 |

Figure 1 shows the photographs of the microstructures produced after heat-forming for one and the same part.

Figure 2 shows the details of the bainites found in castings B, C, D and E.

As shown in Table 2, steels A and G do not reach a strength of 1000 MPa. Steel A has a low percentage of carbon and manganese, such that it does not reach the strength of 1000 MPa or yield strength of 700 MPa. In turn, even though steel G has a higher percentage of carbon and manganese than steel A does, it has a low percentage of silicon, as well as a low percentage of vanadium, such that precipitation hardening is less than in the case of steel A.

Steel F has a tensile strength greater than 1000 MPa and a yield strength of 700 MPa, somewhat greater than steels A and G. However, the mechanical characteristics object of the present patent have not been achieved due to the percentage of carbon at a level that is somewhat below the suitable level.

The compositions of steels B and C were designed as a function of the composition of steel A, but increasing the percentages of manganese in the case of steel B and manganese and silicon in the case of steel C. Therefore, even though strengths exceeding 1050 MPa and yield strengths around 800 MPa were achieved, the percentages of bainite obtained were not acceptable for microalloyed steel with a ferrite-perlite microstructure.

The chemical compositions of steels D and E were subsequently designed, in which in addition to the percentage of carbon, the percentage of manganese of casting B was maintained and the percentages of silicon were increased. However, despite obtaining good mechanical characteristics with strengths greater than 1100 MPa and yield strengths greater than 800 MPa, residual percentages of bainite continued to show up in the different components.

However, for steel H, it has been found that a strength of 1100 MPa can be achieved for bar-shaped parts 30 mm in diameter.

## Claims

1. Microalloyed ferrite -pearlite steel with high tensile strength between 1050 and 1200 MPa and high yield strength greater than 750MPa, comprising the following elements in percentage by weight:
0.35% ≤ C ≤ 0.48%
0.55% ≤ Si ≤ 1.40%
0.55% ≤ Mn ≤ 1.40%
0.05% ≤ V ≤ 0.40%
0.005% ≤ Ti ≤ 0.040%;
0.001% ≤ Nb ≤ 0.050%
the microalloyed steel further comprising optionally at least one of the following elements in percentage by weight:
P ≤ 0.015%
S ≤ 0.10%
Cr ≤ 0.50%
Ni ≤ 0.50%
Mo ≤ 0.10%
Cu ≤ 0.25%
0.001% ≤ Al ≤ 0.050%
0.004% ≤ N ≤ 0.020%
Bi≤ 0.15%
Pb≤ 0.20%
Te≤ 0.02%
Se≤ 0.04%
the rest being iron and impurities.

## Patentansprüche

1. Mikrolegierter Ferrit-Perlit-Stahl mit hoher Zugfestigkeit zwischen 1050 und 1200 MPa und hoher Streckgrenze größer als 750MPa, der die folgenden Elemente in Gewichtsprozent aufweist:
0.35% ≤ C ≤ 0.48%
0,55% ≤ Si ≤ 1,40%
0,55% ≤ Mn ≤ 1,40%
0.05% ≤ V ≤ 0.40%
0,005% ≤ Ti ≤ 0,040%;
0,001% ≤ Nb ≤ 0,050%
wobei der mikrolegierte Stahl ferner wahlweise mindestens eines der folgenden Elemente in Gewichtsprozent aufweist:
P≤ 0.015%
S ≤ 0.10%
Cr ≤ 0,50%
Ni ≤ 0,50%
Mo ≤ 0,10%
Cu ≤ 0,25%
0,001% ≤ Al ≤ 0,050%
0.004% ≤ N ≤ 0.020%
Bi ≤ 0,15%
Pb ≤ 0,20%
Te ≤ 0,02 %.
Se ≤ 0,04%
wobei der Rest Eisen und Verunreinigungen sind.

## Revendications

1. Acier micro-allié de ferrite-perlite de haute résistance à la traction entre 1 050 et 1 200 MPa et de limite élastique élevée supérieure à 750 MPa, comprenant les éléments suivants en pourcentage en poids :
0,35 % ≤ C ≤ 0,48 %
0,55 % ≤ Si ≤ 1,40 %
0,55 % ≤ Mn ≤ 1,40 %
0,05 % ≤ V ≤ 0,40 %
0,005 % ≤ Ti ≤ 0,040 %
0,001 % ≤ Nb ≤ 0,050 %,
l'acier micro-allié comprenant en outre en option au moins l'un des éléments suivants en pourcentage en poids :
P ≤ 0,015 %
S ≤ 0,10%
Cr ≤ 0,50 %
Ni ≤ 0,50 %
Mo ≤ 0,10 %
Cu ≤ 0,25 %
0,001 % ≤ Al ≤ 0,050 %
0,004 % ≤ N ≤ 0,020 %
Bi ≤ 0,15 %
Pb ≤ 0,20 %
Te ≤ 0,02 %
Se ≤ 0,04 %
le reste étant formé de fer et d'impuretés.
